

1

2,925,338

## PHOTOGRAPHIC MASKING USING THE CALLIER EFFECT

Karl H. Schadlich, Binghamton, N.Y., assignor to General Aniline & Film Corporation, New York, N.Y., a corporation of Delaware

No Drawing. Application December 29, 1955  
Serial No. 556,036

4 Claims. (Cl. 96—6)

This invention relates to photography and particularly to a method of producing masked photographic images. More particularly, it relates to the use of the Callier effect in the preparation of corrected color separations.

In the practice of color photography, it is frequently necessary to make prints from color film originals. In making prints, a loss of color saturation occurs, due in large measure, to the imperfect absorption and transmission characteristics of the dyes available for use in color films. For example, the green record is commonly composed of a magenta dye and should modulate and absorb only green light. However, available magenta dye images which are formed in the available color processes have considerable undesired blue and red density and will undesirably modulate and absorb blue and red light to that extent. This same difficulty also exists with respect to the cyan dye images because the cyan dyes formed absorb some of the blue and green light which they are supported to transmit completely. The available yellow dye images are generally closer to ideal and are frequently, although not always, acceptable in regard to color absorption characteristics.

These defects in color absorption are remedied by a masking procedure which consists essentially of making an inverse record of the original dye image processed to a contrast suitable for cancellation of the undesirable density. This inverse record is used combined in registration with the original image to effect the desired cancellation.

Many methods employing color masks have been proposed to satisfy the difference in effective contrast required for the different spectrum bands. In this solution to the problem, the mask image is composed of a dye image to provide the required differential of contrast versus wavelength. The use of dye images for correction masks suffers from the disadvantages of requiring special processing and control methods. Even under optimum conditions, the very nature of the dyes and of the dye images formed renders the color masks less precise than silver masks.

Silver images for masking have the practical advantage of simplicity because the commonly available processing methods provide the needed accuracy of gradient control. Unfortunately, these silver masks are not color selective and, in most instances, several masks must be used since, for example, the undesired blue and red densities of a typical magenta dye are not equal, usually having about twice as much undesired blue density as red density. When correcting the magenta dye spurious densities, one silver mask which is an inverse green record must be used for correcting the undesired blue density when printing the blue separation or record. Another silver mask processed to a lower contrast than the blue mask must be used when printing the red separation or record.

It has also been proposed to use integral silver masks in which a correcting silver image is incorporated in the color film. Of necessity, this type of mask, for

2

instance, the one described in U.S. Patent 2,635,959 provides only a compromise gradient that does not compensate for the differences between the unequal spurious blue and red densities in the magenta layer when used in the usual described manner.

It is an object of this invention to provide a process of masking in which a single silver mask is used to correct completely, two unequal spurious densities in a subtractive dye image which absorbs to a different extent, the two primaries which it is supposed to transmit.

Other objects will be readily apparent from the following description.

I have found that these objects can be accomplished by utilizing the Callier effect to alter and control the effective gradient or printing gamma of a silver mask. By this means, a single silver mask can provide the two gradients required to satisfy optimum masking conditions.

20 The Callier effect, or Q factor, has been known since 1909 and is discussed thoroughly in many photographic texts including Mees' "The Theory of the Photographic Process," revised edition 1954, pages 816-821, and Neblette's "Photography, Its Materials and Processes," 5th edition (1952), pages 250-251. Stated in essence, Callier found that specular light yields maximum density and contrast from a silver image, and the addition of diffusion into the light will reduce the effective density and contrast. The ratio of specular to diffuse density is called the Q factor. This effect is based on the light scattering ability of the silver image. By a suitable selection of a film material for a mask which exhibits a relatively high Q factor, a variety of effective gradients can be effected from a single mask by controlling the 30 degree of diffusion of the printing light source. In general, the effect becomes more pronounced and the Q factor increases with an increase in grain size and density of the silver image.

40 It has already been proposed to use diffuse light for the exposure of the film in which the masking image is formed. This technique results in an unsharp mask which improves the definition of the finished color print but does not affect the effective printing gamma of the mask itself. It has also been proposed to use a vectograph or a silver iodide image for the formation of the mask and to control the amount of correction by adjusting the orientation of the polarizing filter. These methods require not only additional equipment and operations, and are limited to the use of special materials, 45 but also introduce additional sources of error into the reproduction method, and lack the simplicity connected with the use of a simple silver mask.

The essential requirements to utilize my method of masking are as follows.

55 The original color image must have a very low Q factor image so that its contrast will not be affected to any appreciable degree. This requirement is readily met by most color images because the dyes have inherently a very low Q factor. The masking image must have a high Q factor as provided by a silver image of larger grain size so that various degrees of diffusion or collimation of the light will produce relatively effective mask image contrasts.

65 In the production of motion pictures, the following process sequence is commonly used. A color negative film of the integral three-layer type is used for the original photography. From this, direct prints can be made whenever no special effects are required. But, in order to include special effects, to provide additional master negatives, and for other reasons, such as avoiding damage to the original, a duplicate negative is prepared using a

set of separation positives. From these separation positives, a duplicate negative is made which is then used to make the final prints. This duplicate negative, because of the process and printing steps, can include special effects. Inasmuch as the dyes of the original negative display undesired absorption, masking is used in printing the separation positives. Ordinarily, two different masks must be used for the correction of the green record because the blue and red absorptions of the magenta layer are of different magnitudes. In accordance with my invention, the Q factor of the mask is controlled in printing the separation positives, and permits the use of a single mask to correct for the unequal blue and red spurious densities of the color negative magenta image. Similarly, unequal green and blue spurious densities of the cyan dye may be cancelled by the use of a single mask.

The following example will serve to specifically describe the invention as applied to a multilayer color negative film containing color formers. This example should not, however, be construed as limiting or restricting the present invention, but should be considered as merely illustrative.

A multilayer color negative camera film containing color formers is prepared according to the methods described in U.S. Patents 2,179,228, 2,179,239, 2,186,849 and 2,220,187, and consists of an integral tripack emulsion coated on the usual clear cellulose acetate or nitrate film base. Each of the silver halide emulsions is sensitized to one of the primary colors of light, namely, blue, green, and red, and contains a color former fast to diffusion capable of coupling with the oxidation products of an aromatic amino developer to form dyestuff images complementary in color to the sensitivity of the layers. The top layer is blue sensitive and contains p-stearyl amino benzoylacetamino-5-terephthalic acid as a yellow color former. A filter layer, yellow in color and blue absorbing, lies under the top layer. Below this filter layer, lies a green sensitive emulsion layer containing 1-(4'-phenoxy-3'-sulfophenyl)-3-stearyl-5-pyrazolone as the magenta color former. The lowest emulsion layer is red sensitive and contains a mixture of 1-hydroxy-2-naphthoyl-N-octadecylamide-4-sulfonic acid and 1-hydroxy-2-naphthoyl-2'-N-methyloctadecylamino-5'-sulfoanilide as a cyan color former.

The film was exposed in a camera to an original scene and color developed for 15 minutes in a color developer of the following composition:

|                                                 |     |    |
|-------------------------------------------------|-----|----|
| Sodium hexametaphosphate                        | gms | 1  |
| Sodium sulfite                                  | gms | 3  |
| N-ethyl-N-( $\beta$ -hydroxyethyl)amino aniline | gms | 7  |
| Sodium carbonate (monohydrate)                  | gms | 75 |
| Sodium sulfate (anhydrous)                      | gms | 30 |
| Potassium bromide                               | gms | 2  |
| Thallium nitrate, 5% solution                   | ml  | 5  |
| Potassium iodide                                | gms | 3  |
| Water to make 1 liter.                          |     |    |

The developed film was shortstopped for 3 minutes in a bath of the following composition:

|                        |     |    |
|------------------------|-----|----|
| Sodium acetate         | gms | 20 |
| Acetic acid            | cc  | 10 |
| Water to make 1 liter. |     |    |

The shortstopped film was hardened for 5 minutes in a 3% aqueous solution of potassium chrome alum.

After washing for 5 minutes in running water, the film was treated in a bleach bath of the following composition:

|                                      |     |      |
|--------------------------------------|-----|------|
| Sodium hexametaphosphate             | gm  | 0.5  |
| Dipotassium mono-sodium ferricyanide | gms | 100  |
| Sodium acetate (anhydrous)           | gms | 40   |
| Glacial acetic acid                  | ml  | 2.25 |
| Water to make 1 liter.               |     |      |

The developed material was washed for 5 minutes and then fixed for 3 minutes in a solution of the following composition:

|                        |     |     |
|------------------------|-----|-----|
| Hypo                   | gms | 200 |
| Water to make 1 liter. |     |     |

After fixing, the film was washed for 10 minutes in running water and allowed to dry.

A slow speed, fine grain panchromatic film of the type ordinarily used for duplicating black and white negatives was used as the light sensitive material for the preparation of the mask. It was exposed in a contact step printer through the color negative with green light provided by a 3200° K. lamp in combination with a Wratten #61 and a Wratten #15 filter to provide a positive record of the magenta layer. The exposed film was developed to a gamma of .32 (as measured by the Ansco Sweet Densitometer, Model 12) in a developer having the following formula:

|                                     |                                           |      |     |
|-------------------------------------|-------------------------------------------|------|-----|
| 20                                  | Calgon (sodium salt of hexametaphosphate) | gms  | 1.0 |
| Metol (p-methylaminophenol sulfate) | gms                                       | 1.0  |     |
| Sodium sulfite                      | gms                                       | 50.0 |     |
| Hydroquinone                        | gms                                       | 4.0  |     |
| Borax                               | gms                                       | 4.5  |     |
| Boric acid                          | gm                                        | 0.5  |     |
| Potassium bromide                   | gm                                        | 0.25 |     |
| Water to make 1 liter.              |                                           |      |     |

The developing time is 3 minutes at 68° F.

The separation positives are made in an optical printer. The original negative and the raw stock (a fine grain, panchromatic black and white film of the positive duplicating motion picture type) are placed emulsion to emulsion side in contact as a bipack in the camera head side. The mask is used in the projector head side, emulsion side toward the light source. This orientation is used to facilitate registration because it permits mask image size and position adjustments.

The green separation is exposed with green light through the combination of a Wratten #61 and a Wratten #15 filter without the use of a mask. The green separation is developed for a period of 4 minutes in the above black and white developer to a gamma of 0.67.

The blue separation is exposed in registry with the mask through a Wratten #47 combined with an Ansco UV 16P ultraviolet filter. The normally highly collimated light source is used to provide specular light with maximum effective density of the silver image in the mask. The effective gamma of the mask is .43. The blue separation is developed to a gamma of 1.77 which is obtained after 17 minutes of development.

The red separation is exposed in registry with the mask with diffuse light through a Wratten #29 filter. Two plates of ground glass were placed in the beam of the light source to produce the desired diffusion. Measured in diffused light, the mask had an effective gamma of .21. The red separation is processed to a gamma of 1.07 by developing the exposed film for 9 minutes in the above black and white developer.

A balanced set of masked and color corrected separations was obtained which was printed in the conventional manner onto a color negative multilayer film available as Ansco Color Duplicating Negative Type 846 to prepare a duplicate negative. This duplicating film is similar to the camera color negative film except for the use of emulsions of slower speed which is characteristic of duplicating materials.

It will be evident from the foregoing description that, in my masking method, the effective image contrast of the mask depends upon the relative degree or ratio of diffusion or collimation of the printer light; and to a lesser degree, upon the particle size, a factor as expressed by the shape and distribution characteristics of the developed silver in the mask. For maximum utilization of the effect, a high Q factor is desired.

My masking method can also be used to improve the results obtained with an integral silver mask such as the one described in Harsh and Friedman's U.S. Patent 2,635,959. In this method, a mask is formed after color development in the magenta layer utilizing the residual halides which are developed to a silver mask image. When printing from such an integral silver mask color negative, the silver mask will exhibit a Q factor much higher than the dye image. The exposure with red light is carried out with diffusion to produce a relatively lower effective mask contrast while the exposure with blue light is carried out with specular light to produce a higher effective contrast. The green light exposure may be printed with either diffuse or specular light since the mask does not have a color corrective action upon the green record magenta dye, but provides only a contrast reduction. However, the mask has both a color corrective and contrast reducing effect upon the cyan and yellow dye images. Proper compensation for the loss of contrast is accomplished by increasing the layer contrasts of the negative, the positive or both. In this manner, only the dual color correction effect of the mask is retained without any loss of contrast.

While I have herein disclosed the preferred embodiments of my invention, I do not desire to limit myself solely to the foregoing illustrative example, since it will be readily apparent to those skilled in the art that the foregoing procedural steps may be varied and other similar steps and processing solutions employed without departing from the spirit and scope thereof. For example, a positive record of the cyan image can be used to correct for unequal spurious absorptions of the blue and green primaries by the cyan layer. In this case, the red record is printed with red light without the use of a mask while both the green and blue records are printed in registration with the silver mask using specular light for the primary requiring a higher effective mask contrast and using diffuse light for the other primary requiring a lower effective mask contrast.

Instead of color formers fast to diffusion, there may be used a multicolor film in which each element bears a color yielding layer comprising a hydrophilic, film-forming synthetic polymer containing a plurality of hydroxyl groups and having a plurality of color components and, in addition, containing light sensitive silver salts as described in U.S. Patents 2,397,864, 2,397,865, 2,397,866 and 2,397,867. Accordingly, therefore, only such limitations should be imposed as are indicated in the following claims.

I claim:

1. The method of making color corrected color separation positives from a multilayer subtractive color negative containing in the magenta layer, a magenta dye image having, in addition to the green absorption density, an undesired absorption density for blue and an undesired absorption density for red, the undesired density of blue being greater than the undesired density of red, which includes the steps of preparing a positive color correction silver masking image which is a positive record of the magenta image, placing the silver mask in registry with said multicolor negative and printing the masked negative onto a black and white film while changing the effective printing gamma of the silver mask by using a collimated blue light for the printing of the blue separation, and a diffused red printing light for the printing of the red separation, the degree of diffusion of said red printing light being such as to equalize the effective printing gamma of the silver correction mask with the gamma of the undesired absorption density for red.

2. The method of preparing color corrected color separation positives from a multilayer subtractive negative

containing in the several layers, yellow, magenta and cyan part images in which the yellow part image does not require correction, in which the magenta part image absorbs, in addition to green, also lower and undesired densities of blue and red, the undesired density of blue being greater than the undesired absorption of red, and in which the cyan image absorbs, in addition to red, also the primaries green and blue, which includes the steps of preparing a positive color correction silver mask by exposing a light sensitive silver halide film with green light through the negative and developing the exposed film to a silver positive, placing the mask thus obtained in registry with the multicolor negative and printing the blue separation with specular blue light, and printing the red separation with diffused red light, the degree of diffusion of said red printing light being such as to equalize the effective printing gamma of the silver correction mask with the gamma of the undesired density of red.

3. The method of making color corrected color separation positives from a multilayer subtractive color negative containing in the cyan layer, a cyan dye image having, in addition to the red absorption density, an undesired absorption density for blue and an undesired absorption density for green, the undesired density of blue being greater than the undesired density of green, which includes the steps of preparing a positive color correction silver masking image which is a positive record of the cyan image, placing the silver mask in registry with said multicolor negative and printing the masked negative onto a black and white film while changing the effective printing gamma of the silver mask by using a collimated blue light for the printing of the blue separation, and a diffused green printing light for the printing of the green separation, the degree of diffusion of said green printing light being such as to equalize the effective printing gamma of the silver correction mask with the gamma of the undesired absorption density for green.

4. The method of preparing color corrected color separation positives from a multilayer subtractive negative containing in the several layers, yellow, magenta and cyan part images in which the yellow part image does not require correction, in which the cyan part image absorbs, in addition to red, also lower and undesired densities of blue and green, the undesired density of blue being greater than the undesired absorption of green and in which the magenta image absorbs, in addition to green, also the primaries red and blue, which includes the steps of preparing a positive color correction silver mask by exposing a light sensitive silver halide film with red light through the negative and developing the exposed film to a silver positive, placing the mask thus obtained in registry with the multicolor negative and printing the blue separation with specular blue light, and printing the green separation with diffused green light, the degree of diffusion of said green printing light being such as to equalize the effective printing gamma of the silver correction mask with the gamma of the undesired density of green.

#### References Cited in the file of this patent

#### UNITED STATES PATENTS

|           |               |                |
|-----------|---------------|----------------|
| 2,294,981 | Hanson        | Sept. 8, 1942  |
| 2,360,225 | Hanson et al. | Oct. 10, 1944  |
| 2,384,612 | Evans et al.  | Sept. 11, 1945 |
| 2,458,437 | Smith         | Jan. 4, 1949   |
| 2,543,706 | Pohl          | Feb. 27, 1951  |

#### OTHER REFERENCES

Mees: "The Theory of the Photographic Process," revised edition, Macmillan Co., N.Y., 1954, page 818.  
(Copy in Scientific Library.)